

# UNITED STATES PATENT OFFICE.

JAMES LOCKHART JARDINE, OF PENICUIK, SCOTLAND.

## PROCESS FOR THE PRODUCTION OF PAPER-PULP OR CELLULOSE FROM BAMBOO AND THE LIKE.

1,143,401.

Specification of Letters Patent. Patented June 15, 1915.

No Drawing.

Application filed August 6, 1914. Serial No. 355,473.

To all whom it may concern:

Be it known that I, JAMES LOCKHART JARDINE, a subject of the King of Great Britain and Ireland, and a resident of Penicuik, Midlothian, Scotland, have invented a certain new and useful Process for the Production of Paper-Pulp or Cellulose from Bamboo and the like, of which the following is the specification.

10 A commercially bleachable pulp cannot be produced from bamboo or similar vegetable growths the incrusting ingredients of which are mixtures of lignin and pectose, or substances chemically similar, by any of the 15 bisulfite processes as employed for extraction of pulp from wood and the like lignified substances. I have discovered that this is due to the excessive acidity of the liquor as used in the process of digestion, caused 20 by the liberation and retention in the digester of the sulfurous acid gas.

At present in the wood pulp process where the digester is internally heated, the sulfurous acid gas liberated in the heating and 25 cooking is, as far as practicable, kept in contact with the pulp, and only quantities are allowed to escape from the digester sufficient to admit of the entrance of enough steam to 30 secure and maintain the proper cooking temperature, this being controlled by direct thermometer readings.

If bamboo and the like be treated in a similar manner, a secondary reaction occurs in the later stages of the cooking which upsets the chemical equilibrium and a brown aldehydic product is deposited on the fibers, rendering them commercially unbleachable, or if the hydrolysis is lessened to prevent 35 the deposition of this organic reducing 40 agent the resolution is incomplete, and although a light yellow colored pulp can be secured it does not bleach as the fibers are still combined with or incased in incrusting ingredients.

45 My invention consists in a process whereby these difficulties are overcome, my method insuring that the ligno and pectic constituents, along with the coloring matters, and the like, are so thoroughly removed that the 50 subsequent bleaching for the production of a white pulp does not need more of the usual bleaching agents than are required for pulps already used in the trade.

In the process forming the subject matter 55 of the present invention, a base which yields

a soluble sulfite must be selected, such as magnesium, or sodium, or their equivalents, and to it is added in any convenient manner sulfurous acid gas as in certain known processes for the resolution of wood, but according to the invention these chemicals are so used for the production of paper pulp from bamboo and the like that the deposition of an aldehyde is prevented and only the proper degree of acidity is maintained to 60 sulfonate the lignin, leaving the base free to resolve the pectic and coloring ingredients.

Magnesia does not readily dissolve in weak sulfurous acid, and thus when its solution is effected by any of the ordinary processes, the resultant liquor generally shows at least the bisulfite proportions of  $\text{SO}_2$ . Sodium sulfite on the other hand is readily soluble, and a solution containing approximately three-fifths of the bisulfite equivalent 70 provides a liquor with a surplus of available  $\text{SO}_2$ , so rendering it suitable for my process. Such a solution may contain about five atoms of sodium to three of sulfur.

In order that the fibrous tissues may rapidly and uniformly absorb the liquor, their colloidal adhesions must be broken down by mechanical crushing. The raw material after receiving this preliminary treatment is packed in a digester, the prepared liquor is 75 added, and the heating and cooking is secured by the application of direct steam.

It is advisable not to fill the digester too full, as space is necessary for the free separation of the gases evolved from the liquor, 80 and as these are liberated they must at once be removed; and for this purpose a continuously free exhaust fixed in the highest part of the digester is kept open throughout the entire cooking. The escaping steam and gas 85 may be passed to a cooling coil or condensing apparatus for  $\text{SO}_2$  recovery in any known manner.

So thoroughly must the gasified  $\text{SO}_2$  be removed that no opposing pressure is created in the digester; the cooking temperature is thus at all stages directly equivalent to the steam pressure, and no thermometer need be used.

The stage of resolution is easily determined by a test of the total sulfurous acid percentage contents of the liquor, and as the reduction of this toward the finish of the cooking is gradual, the most advantageous point of exhaustion can be secured. 105

Throughout the digestion by the removal of the gasified  $\text{SO}_2$  the degree of active acidity automatically regulates itself to suit the condition of the pulp and the holding capacity of the base; thus there are no complications, and resolution proceeds along regular lines.

To secure the complete removal of the encrusting ingredients, or complete decortication, sufficient free or available sulfurous acid to sulfonate the lignin must be provided, and as variations in the proportions of this substance occur, it is advisable to have excess sulfurous acid in the liquor at the start of the digestion, the surplus being liberated and readily removed in the manner already described. Or the excess may be otherwise removed.

Any increase in the proportion of the pectose constituents requires a corresponding increase in the percentage of the base, but under all conditions excess of this must be provided, as it insures complete resolution and the consequent slow reduction of the liquor strength in the last stages of the cooking.

Having enumerated the principles of my invention, I now give working details of a method as applied to the common bamboo of the West Indies. This bamboo must be very thoroughly and uniformly crushed, cut into convenient lengths, and packed into a vertical digester with acid proof lining. Between 10 and 12 lbs. of the crushed material can easily be packed into each cubic foot capacity of the digester, and about one gallon of liquor is required for two lbs. of bamboo, or on the weight basis this means roughly five to one. A suitable liquor made in a known manner from a magnesium base gives the following  $\text{SO}_2$  analysis:—

|                           |       |
|---------------------------|-------|
| Total $\text{SO}_2$ ----- | 3.25% |
| Available or free-----    | 1.80% |
| Combined-----             | 1.45% |

After placing the bamboo and liquor in the digester, the lid is fixed and a small exhaust pipe connection is made to a cooling coil which has a free outlet into an absorption apparatus forming part of the liquor-making plant. The steam is applied to the digester, and the full gage pressure of 75 lbs. or 5 atmospheres is reached in three to four hours. The air and surplus sulfurous acid come off very rapidly during the heating up of the contents, and the full capacity of the outlet is then required; but thereafter, to prevent steam waste, it can be curtailed by partially shutting the outlet control cock. The rate of gas liberation in the further stages of the cooking is relatively slow, and thus a smaller outlet is sufficient. Under these circumstances the condensation of steam in the cooling coil during the cook-

ing amounts to 15%, or 20% of the volume of the liquor added, and the sulfurous acid recovered is 20% to 25% of the original.

The removal of the surplus or gasified  $\text{SO}_2$  is necessary for the chemical reasons already stated, for if this is not thoroughly effected the acid unduly preponderates, preventing the alkaline base from having freedom to remove the pectose constituents, or completely upsetting the chemical equilibrium and depositing the aldehyde.

Care must therefore be taken to insure that all the gasified  $\text{SO}_2$  escapes from the liquor, and to a certain extent the process can be hurried by arranging for a larger steam escape in the later stages of the cooking, as this more rapidly carries off the traces of free  $\text{SO}_2$ , allowing the base to more quickly effect the removal of the coloring and gummy substances.

After reaching full pressure, ten to twelve hours are required to complete the cooking process, this being carried on until the percentage of total sulfurous acid in the liquor, as ascertained by direct test with standard iodin solution, is very much reduced. A suitable and satisfactory final strength, where dry steam has been used, is about .1%. When this stage is reached the steam is shut off, and that contained in the digester is either blown out direct to atmosphere, or it can be condensed through a cooling coil, though the latter process is not necessary from the point of view of sulfur economy, seeing the bulk of this element which is not required in the chemical action has already escaped and been recovered. After the pressure has been sufficiently reduced, the contents of the digester are blown out, and the resultant pulp is of a grayish-white color. The yield is fully 50% of the original weight of bamboo furnished.

The pulp can be bleached by ordinary methods to a full white with about 12% of bleaching powder calculated on the dry weight of pulp.

What I claim is:—

1. A process of producing easily bleachable paper pulp from bamboo and the like, which comprises cooking said material, in a crushed condition, under pressure, with a solution of a water-soluble sulfite containing, at the commencement of the cook, an excess of available  $\text{SO}_2$  over the amount necessary to form normal sulfite, and maintaining said liquor, during the latter part of the cook, substantially free from uncombined  $\text{SO}_2$ , by relieving the gas pressure at such a rate that substantially all the liberated  $\text{SO}_2$  is drawn off, and thereby prevented from accumulating in the liquor.

2. A process of producing easily bleachable paper pulp from bamboo and the like, which comprises cooking said material, in a

crushed condition, under pressure, with a solution of magnesium bisulfite containing, at the commencement of the cook, an excess of available SO<sub>2</sub> over the amount necessary 5 to form normal sulfite, and maintaining said liquor, during the latter part of the cook, substantially free from uncombined SO<sub>2</sub>, by relieving the gas pressure at such a rate that substantially all the liberated

SO<sub>2</sub> is drawn off, and thereby prevented 10 from accumulating in the liquor.

In testimony whereof I have signed my name to this specification, in the presence of two subscribing witnesses.

JAMES LOCKHART JARDINE.

Witnesses:

WILFRED HUNT,  
JAMES EAGLESOM.